

# UNITED STATES PATENT OFFICE.

JOHN H. PFINGSTEN, OF MILWAUKEE, WISCONSIN, ASSIGNOR TO PRESTO COLOR COMPANY, OF CUDAHY, WISCONSIN.

## COLOR-BASE FOR LEATHER-FINISHES AND METHOD OF MAKING THE SAME.

1,393,697.

Specification of Letters Patent.

Patented Oct. 11, 1921.

No Drawing.

Application filed May 28, 1921. Serial No. 473,361.

To all whom it may concern:

Be it known that I, JOHN H. PFINGSTEN, a citizen of the United States, residing in Milwaukee, county of Milwaukee, and State of Wisconsin, have invented a certain new and useful Improvement in a Color-Base for Leather-Finishes and Method of Making the Same, of which the following is a specification.

10 During the process of tanning and before the leather is ready for the market it is necessary to apply different surface finishes to give the requisite colors, etc. In the past these have been made up in liquid form, are 15 very bulky, expensive to transport, and are for the main part easily putrescible as they contain binders consisting of gelatin, casein, and similar animal and vegetable products which decompose very rapidly, consequently 20 it is necessary to put in preservatives such as arsenic, oil of mirbane, etc., which are dangerous to the workers unless used in very minute quantities, and in some cases are foul smelling. 25 The leather finishes as heretofore sold contain approximately 80 per cent. of water. It is in paste form containing all the essentials of the leather finish with the exception of the water and the binder. I am thus enabled to get a concentrated base of a concentration of at least ten to one. One gallon of my invention will make the color base for 30 ten gallons of finish. It is easy to handle, does not leak, need not be hermetically 35 sealed, will not freeze, and contains no substantial amount of active poisonous preservative.

With these and other objects in view my invention consists in the following combination of ingredients. I have found that it is impractical to make a color base for finishing leather in paste form following the methods heretofore in use. It is imperative that the colors be very finely ground so as 45 to be finely pulverulent. This cannot be accomplished by ordinary means by grinding in water as a sufficient degree of pulverization cannot be obtained. Neither can it be accomplished by grinding in oil as is the case 50 in paints, as the finish must be used by mixing with water, and oil and water are practically immiscible. I have therefore discovered that by using a combination of a sulfonated oil such as Turkey red oil, which

is water soluble, thinned somewhat with 55 water, will give me a practical grinding vehicle which will not only enable me to grind my pigments to the proper degree of fineness but will also give me a resultant product which as to the vehicle is water soluble. The 60 pigments being very finely divided are easily held in suspension when in use, they are almost in a colloid condition.

In preparing my base for leather finish I take a suitable mixture of pigments which 65 will give me the desired shade, such for instance as chrome yellow—ten pounds, French ocher—two pounds. This is then mixed with three pounds of water and three pounds of sulfonated oil and ground to an extremely 70 fine consistency in an ordinary painter's stone mill. The material is then ready for packing and I may either pack it in tin containers and sterilize the container, including the contents, or may add a very small 75 amount of preservative such as 1/100th of one per cent. of mercuric chlorid to prevent the forming of mold. Paradoxical as it may seem, I have found that this product when made up is subject to mold and I have finally 80 discovered that 1/100th of one per cent. of mercuric chlorid will counteract the tendency of mold and give a perfectly stable product. The product so prepared is ready 85 for use by simply mixing with water and a binder, such as Irish moss, casein, blood albumin, shellac etc., and is of course to be kept constantly agitated as is customarily done with all finishes of this sort.

My invention has the advantages of permanency, safety, extreme concentration, freedom from freezing, from putrescible, saving in bulk, may be made up in exact amounts as wanted by the purchaser, is odorless, and contains oxidizing agents, i. e., a sulfonated 90 oil, which gives the paint-like characteristic to the mixture, i. e., it dries by oxidation and not by evaporation and at the same time it is water soluble.

Having fully disclosed my invention, I 100 claim:

1. A concentrated color base suitable for making leather finishes which consists of a pigment and a water soluble oil, the pigment being so finely divided as to be in substantially a colloid condition when diluted with water.

2. A concentrated color base suitable for

making leather finishes, which consists of a finely ground pigment, water soluble oil, and water, and a preservative against mold.

3. A concentrated color base suitable for 5 making leather finishes, which consists of a finely ground pigment, water soluble oil, and water, and containing a small amount of mercuric chlorid.

4. The method of preparing a pigment 10 color base for leather finishes which consists in grinding the pigment in a solution of a water soluble oil and water to pulverulent form, putting the same in containers and sterilizing the containers and contents 15 thereof.

5. The method of preparing a pigment color base for leather finishes which consists in grinding the pigment in a solution of a water soluble oil and water to pulverulent form, and adding a preservative against 20 mold.

6. The method of preparing a pigment color base for leather finishes which consists in grinding the pigment in a solution of a sulfonated oil and water to pulverulent 25 form, putting the same in containers and sterilizing the containers and contents thereof.

JOHN H. PFINGSTEN.